

## UNITED STATES PATENT OFFICE

GUSTAVE DANIEL FORTMAN, OF PHILADELPHIA, PENNSYLVANIA

## LEATHER COMPOSITION

No Drawing.

Application filed March 21, 1928. Serial No. 263,603.

In every process of manufacture of articles of leather, for instance, shoes, belts, trunks, suitcases, hand bags, etc., there is a large percentage of clippings too small to make any leather article, and such leather scrap is wasted except as it may be utilized for fertilizer or made into charcoal for heat treatment of ferric metals. It is the object and effect of my invention to utilize such leather scraps, for any purpose for which the original leather web may be used, by uniting such scraps in substantially homogeneous webs, or other forms; the process of my invention hereinafter described being operative to not only produce leather compositions respectively resembling the various commercial forms of natural leather, having various degrees of hardness and flexibility, but to produce other compositions which are much harder and more durable than any natural leather and more in the nature of horn.

In effecting my invention, I prefer to grind, or otherwise comminute, the leather scraps to such a degree that a mass thereof seems to be of uniform texture when passed between the fingers of the operator, for the reason that when reduced to such state, the product is smoothly homogeneous. However, it is unnecessary to thus uniformly comminute the leather ingredients of my composition, which may be in the form of irregular shreds mixed with flocculent particles, or otherwise. However, when the leather is used in such irregular form, there are corresponding irregularities in the product, but that is desirable for production of webs having an irregular, instead of a smooth, surface.

The comminuted leather, in any form above contemplated, is integrated in a tenaciously coherent, more or less elastic and flexible web or other form by a binding medium which is primarily a liquid but which solidifies in the product to a tough horn-like substance extending between and uniting the particles of the leather in a substantially homogeneous mass. However, it is characteristic of all of the products of my invention herein contemplated that the outer surfaces thereof are smoothly unctuous like natural leather, as distinguished from artificial leather compo-

sitions of the prior art which are sticky; my products being tenaciously coherent and cohesive, but not adherent or adhesive, to anything with which they come in contact.

I have found it convenient to make such binding material by mixing commercial cottage cheese with commercial aqua ammonia in the proportion of five pounds of cheese to one pint of the ammoniacal liquid. The effect of thus alkalinating the cheese is to more or less saponify the fatty constituents thereof. After that mixture has been allowed to stand for about two hours, I thoroughly mix one ounce of hydrochloric acid therewith. Such acidulation of the mass substantially neutralizes its alkalinity. The addition of the acid causes a chemical reaction with the ammonia throughout the mixture with production of fumes which are extremely acrid and should be avoided by the operator. When such reaction is completed, the mass is allowed to dry and, when dried, resembles horn; being principally gelatinized casein. That dried material is then dissolved in benzol (a hydrocarbon distillate of petroleum otherwise known as benzene  $C_6H_6$ ), until it forms a gummy liquid, the viscosity of which varies with the proportion of the solid matter dissolved in the hydrocarbon.

The leather, in any comminuted form above contemplated, is then mixed with the gummy binding liquid aforesaid in such proportions as to coat the particles of leather and form a film between them when they are pressed together in a dough-like mass, which may be kneaded or otherwise manipulated or agitated until of substantially uniform consistency. The resulting plastic mass may then be rolled or pressed to form a plane sheet or web of any desired extent, or may be otherwise shaped by hand, or in a mold, or by any other suitable means, and may be permitted to dry spontaneously by evaporation of the hydrocarbon, or may be warmed to accelerate its desiccation. The residue of the binding medium above described is pliable and more or less elastic, but harder than the leather particles mixed therewith. Consequently, the degree of hardness of the prod-

uct may be determined and varied in accordance with the proportion of the binding material residue left in a given mass of comminuted leather. For instance, from the same comminuted leather, I may produce a thin flexible web resembling soft tanned calf-skin, such as is used for shoe uppers; or a thicker, harder and tougher web resembling sole leather; the latter having more binding material per unit of volume than the soft product aforesaid.

Moreover, the degree of hardness of a given composition of leather and binding material may be increased by forming the product under water, which penetrates the leather particles and, when evaporated, leaves such particles in a harder, stiffer state than particles which have not been wet; such hardening effect being similar to that produced upon natural leather by wetting and drying it.

Although I find it convenient to mix the composition aforesaid of the consistency of dough for the formation of webs thereof by rolling or pressing means; I do not desire to limit myself to that method of procedure, for a composition in accordance with my invention may be primarily of the consistency of paint so that it may be spread to the desired form by a brushing operation. Such paint-like consistency is attained by the use of more of the hydrocarbon solvent of the casein than is used in the composition of a dough-like consistency. In other words, the viscosity of the mixture may be varied at the convenience of the operator in accordance with the proportion of the solvent employed. However, the solvent being volatile, the consistency of the resulting product is determined by the proportion of the solute which is left in the composition and not by the quantity of the volatile solvent, which is merely a convenient medium for manipulating the residual ingredients during the process of manufacture of the products aforesaid.

It is characteristic of all of the compositions of my invention herein contemplated that they are water-proof, in the sense that they are not disintegrated by immersion in water. Moreover, they are so far resistant to the action of electricity as to be classed as dielectrics.

Although I have found it convenient to use commercial cheese as the source of the casein ingredient of my composition; of course, I may produce casein directly from cow's milk by skimming the cream therefrom; allowing the skimmed milk to stand in a warm place until it curdles; then separating the curds from the whey by percolation through a filter, of paper or other suitable material, and washing the curds with water to eliminate the lactic acid therefrom.

Then the curds may be wrapped in a cloth

and boiled to remove the fat, and dried to a horn-like consistency; such residue being substantially pure casein.

Although I have found it convenient to produce the binding material aforesaid from casein which is formed by first alkalinating and then acidulating and then desiccating milk curds, I do not desire to limit myself to casein thus produced. Moreover, although I prefer to use the high grade hydrocarbon benzol, it is much more costly than the similar hydrocarbons, of varying composition, which are known to the trade as benzine and which may be used as a solvent of gelatinized casein to produce a binding material of the general character above contemplated.

I am aware that it is not new to form a cementitious material of gelatinized casein. However, the heretofore known solvents of such casein, such as strong acids, alkalis, and sodium silicate etc., are of such nature as to prevent their use in any composition which is to resemble leather. So far as I am aware, it is broadly new, and original with myself, to form a solution of gelatinous casein in benzol or any similar hydrocarbon distillate; the characteristic of which is that it volatilizes from the product leaving the casein as a flexible binding medium integrating the primarily separate and distinct particles of leather in a substantially homogeneous mass resembling natural leather, in all of the physical qualities of the latter, including such surface tension as to render the surface thereof unctuous like natural leather, without any tendency to adhere to anything with which it comes in contact.

Therefore, I do not desire to limit myself to the precise details of the process or product herein set forth, as it is obvious that various modifications may be made therein without departing from the essential features of my invention, as defined in the appended claims.

I claim:

1. A composition of matter, which is non-corrosive and inodorous, including comminuted leather particles comminuted to such a degree that a mass thereof seems to be of uniform texture when passed between the fingers of the operator, said particles being connected by a binding medium including the residue of casein alkalinated and acidulated to a chemically neutral state and dissolved in a volatile hydrocarbon.

2. A composition of matter, which is non-corrosive and inodorous, including comminuted leather particles comminuted to such a degree that a mass thereof seems to be of uniform texture when passed between the fingers of the operator, said particles being connected by a binding medium including the residue of casein alkalinated and acidulated to a chemically neutral state and dissolved in benzol.

3. The process of forming a leather composition which is noncorrosive and inodorous, and which includes mixing cottage cheese with aqua ammonia in the proportions of five pounds of cheese to one pint of ammonia liquor; then adding hydrochloric acid and agitating the mixture until it is substantially uniform and in a chemically neutral state; allowing said mass to dry; 5 dissolving the dried mass in benzol until it forms a gummy binding liquid; then mixing said binding liquid with a mass of comminuted leather particles comminuted to such a degree that a mass thereof seems to 10 be of uniform texture when passed between the fingers of the operator; shaping the product to the desired form and desiccating it.

4. The process of forming a leather composition which is noncorrosive and inodorous, and which includes mixing cottage cheese with sufficient aqua ammonia to saponify the fatty constituents of the cheese; then adding hydrochloric acid to neutralize the 20 alkalinity of the mass and agitating the mixture until it is substantially uniform; allowing said mass to dry; dissolving the dried mass in a volatile hydrocarbon distillate of petroleum until it forms a gummy binding 25 liquid; then mixing said binding liquid with a mass of comminuted leather particles comminuted to such a degree that a mass thereof seems to be of uniform texture when passed between the fingers of the operator; shaping the product to the desired form and desiccating it.

5. The process of forming a leather composition which is noncorrosive and inodorous, and which includes dissolving gelatinous casein in a volatile hydrocarbon, forming a gummy binding liquid; and then mixing said binding liquid with a mass of comminuted leather particles comminuted to such a degree that a mass thereof seems to 40 be of uniform texture when passed between the fingers of the operator.

6. The process of forming a leather composition which is noncorrosive and inodorous, and which includes dissolving gelatinous casein in benzol, forming a gummy binding liquid; and then mixing said binding liquid with a mass of comminuted leather particles comminuted to such a degree that a mass thereof seems to be of uniform texture when passed between the fingers of the operator.

In testimony whereof, I have hereunto signed my name at Philadelphia, Pennsylvania, this nineteenth day of March, 1928.

GUSTAVE DANIEL FORTMAN.